# EUROPEAN PATENT SPECIFICATION

(11) **EP 0 161 579 B1**
(45) Date of publication and mention of the grant of the patent: **07.02.1990**
(21) Application number: 85105288.6
(22) Date of filing: 30.04.1985
(51) Int. Cl.: D21F 1/00

(54) **Dryer fabric having warp strands made of melt-extrudable polyphenylene sulphide**
Trockengewebe mit Kettenfäden aus schmelzextrudierbaren Polyphenylensulfiden
Toile de séchage comprenant des fils de chaîne en polyphénylène sulphide extrudable au fondu

(30) Priority: 01.05.1984 US 605825; 26.04.1985 US 727665
(43) Date of publication of application: 21.11.1985
(73) Proprietor: JWI Ltd., Kanata, Ontario (CA)
(72) Inventor: Baker, Samuel M., Carleton Place, Ontario K7C 1M1 (CA); Best, F. Brian, Ottawa, Ontario K2A 3J6 (CA); Bhatt, Girish M., Williston Vermount 05495 (US)
(74) Representative: Dipl.-Phys.Dr. Manitz Dipl.-Ing. Finsterwald Dipl.-Ing. Grämkow Dipl.Chem.Dr. Heyn Dipl.Phys. Rotermund Morgan, B.Sc.(Phys.)

(56) References cited:
- EP-A- 0 063 380
- EP-A- 0 070 708
- FR-A- 2 418 826
- US-A- 4 267 227
- US-A- 4 290 209

## Description

### Background of Invention

### (a) Field of the Invention

The present invention relates to fabrics made of synthetic materials and particularly, but not exclusively, for use in dryer sections of papermaking machines involving high temperature. Furthermore the present invention relates to monofilaments suitable for use in such fabrics.

### (b) Description of Prior Art

Increasingly dryer fabrics are being manufactured from monofilament strands because such fabrics are easier to keep clean, thus retaining their drying efficiency, and because they are essentially non- absorptive. These are normally of woven construction, but in recent years an alternative non-woven construction is becoming popular - the so-called "spiral fabrics" - which are assembled from a multiplicity of helical coils connected together by inserted hinge pins. German patent DE 24 19 751 and U.S. 4,481,079 described this type of fabric. The predominant material used in such fabrics, whether woven or spiral, is polyester, with polyamides used less frequently. Unfortunately both of these classes of materials degrade at high temperature, a short-coming which precludes their use in high temperature applications on paper machines. High temperature applications are ones that result in operating temperatures of about 150°C or above.

Some manufacturers of woven fabrics have resorted to NOMEX^{O} or KEVLARO in order to cope with the extreme conditions prevalent in such high temperature applications. Because neither polymer is mett- extrudable, monofilaments made from them are not practicable and so these materials are employed in the form of composite multifilaments, often resin coated. U.S. 4,159,618 teaches such a monofilament-like composite strand for this purpose, but even these composites are deficient in that they lose tensile strength when exposed to moist or dry heat (see Tables 1-3 in U.S. 4,159,618).

Considering now another property of dryer fabrics, it is highly desirable that such fabrics be distortion resistant, that is, have inherent dimensional stability and retain this property so as to resist skewing throughout their life on the paper machine. Woven fabrics made with monofilament warp of round cross-section, and conventional materials such as polyester while having the desirable advantages of running clean and of non-absorptivity already mentioned, are generally deficient in distortion resistance because of the minimal interlocking contact at the warp and weft cross-overs dictated by the geometry of the respective strands. U.S. 4,290,209 discloses the use of rectangular cross-section warp strands having a flattening ratio of about 2:1, whereby the resulting fabric acquires superior properties of distortion resistance and surface smoothness, along with more desirable permeability and elastic modulus. None of these improved fabrics, however, are suitable for high temperature applications, again because of the inherent tendency of the polymers normally used to degrade and lose strength.

U.S. 4,359,501 discloses an industrial fabric, for use in applications involving elevated temperatures, comprised of melt-extrudable polyaryletherketone monofilament strands. This material, however, suffers the major disadvantage of being so costly that the woven end product is not economically attractive to the specific paper mill end-users already identified.

The present invention is directed towards solving these problems.

### Summary of the Invention

Broadly, the present invention provides a dryer fabric for use in a dryer section of a paper machine wherein at least the machine direction components of the fabric are monofilaments made from polyphenylene sulphide or a blend of polyphenylene sulphide with heat-stabilized polyamide 66 with the polyamide 66 being present in the range of up to about 20% by night.

In a preferred embodiment of the invention the polyphenylene sulphide is blended with about 6% by weight of heat-stabilized polyamide 66.

In another preferred embodiment the dryer fabric comprises a plurality of interwoven warp and weft strands wherein at least the warps are monofilaments made from polyphenylene sulphide or a blend of polyphenylene sulphide with heat-stabilized polyamide 66 the warp strands having an essentially rectangular cross-section with the long axis of the rectangle lying in the plane of the fabric.

In another preferred embodiment the dryer fabric comprises a multiplicity of helical coils connected together by hinge pins wherein at least the helical coils are made from polyphenylene sulphide or a blend of polyphenylene sulphide with heat-stabilized polyamide 66.

In another preferred embodiment the dryer fabric comprises a multiplicity of helical coils connected together by hinge pins wherein at least the helical coils are made from polyphenylene sulphide or a blend of polyphenylene sulphide with heat-stabilized polyamide 66 and wherein the helical coils have an essentially rectangular cross-section when viewed in the machine direction with the long axis of the rectangle lying in the plane of the fabric.

The present invention also comprises a monofilament as set forth in claim 12 and a synthetic fabric made therefrom. Further advantageous embodiments of the invention are defined in the subordinate class.

The present invention thus recognizes that monofilaments of the type described above can also be used to advantage in other industrial applications where hydrolysis is encountered. For the sake of completeness it should be pointed out that polyphenylene sulphide fibres are known per se as can be seen from U.S. patent 3,919,177. However, this disclosure does not recognize the property of polyphenylene sulphide monofilaments which is of importance here, namely the resistance to hydrolytic degradation at elevated temperatures. Another publication describing polyphenylene sulphide fibres is the preliminary bulletin of Phillips Petroleum Company issued in Feb. 1983 describing their "Ryton" (Registered Trademark) product. Although this publication demonstrates the chemical inertness of polyphenylene sulphide, it was the present applicants who first proved that a PPS monofilament was immune to hydrolytic attack.

### Brief Description of Drawings

Fig. 1 is a schematic view of a typical dryer section as used in a papermaking machine;
Fig. 2 is an enlarged sectional view of an all-monofilament plain weave dryer fabric utilizing flattened warp strands;
Fig. 2A is a fragmented sectional view along section line A-A of Fig. 2;
Fig. 3 is an enlarged sectional view of an all-monofilament four-shaft eight-repeat duplex-weave dryer fabric utilizing flattened warp strands;
Fig. 3A is a fragmented sectional view along cross-section line A-A of Fig. 3.
Fig. 4 is an enlarged cross-section view of the flattened warp strand;
Fig. 5 is a plan view of a part of a spiral dryer fabric with flattened spirals; and
Fig. 5A is an enlarged sectional view, along cross-section line A-A of Fig. 5, of the spiral fabric viewed in the machine direction.

### Detailed Description of the Invention

Referring to Fig. 1 there is schematically illustrated a sub-section of a typical dryer section in a papermaking machine (not shown). The top tier dryer cylinders are generally indicated at 10 and the bottom tier at 11. The paper web 13 passes in a serpentine fashion over the top and bottom dryer cylinders as shown. An endless top fabric 14 holds the paper web 13 tightly against the upper cylinders 10 as it passes partially around the first upper cylinder, around a felt roll 15, partially around the remaining top cylinders 10 and around the other intervening felt rolls 15, then around return roll 16, passing over guide and tensioning rolls 24 and 23 respectively, and then over other return rolls 16 before it passes again over the first dryer cylinder to complete the cycle. Similarly, an endless bottom fabric 18 holds the paper web 13 tightly against the lower dryer cylinders 11 as it passes around these and the intervening bottom felt rolls 19, return rolls 21, tensioning roll 25, guide roll 26, and other return rolls 21, substantially as shown.

Polyphenylene sulphide is a linear high molecular weight polymer having the repeating unit and is available commercially under the registered trademark RYTON from Phillips Chemical Corporation. While priced at a fraction of the material of U.S. 4,359,501, pure polyphenylene sulphide of the present invention is difficult to extrude. It is also lacking in "toughness" required for industrial weaving.

We have found that monofilament polyphenylene sulphide has greatly superior resistance to hydrolytic degradation than the polyester strands commonly used in dryer fabrics. Table 1 shows the results of a test with the percent retained tensile strength of a polyphenylene sulphide strand exposed to saturated steam at 130°C in a pressure vessel (24 gauge psi) for a period of eight days, along with a polyester monofilament strand of the same size.

Table 2 shows test results for the same materials when exposed to saturated steam at 150°C.

It will be observed that in these accelerated tests the strength of the polyphenylene-sulphide strand was not only retained but was, in fact, enhanced whereas the polyester strand showed a rapid and catastrophic loss in strength. This extraordinary retention of hydrolysis resistance, even after prolonged exposure, makes polyphenylene sulphide an outstanding candidate material for use in paper machine dryer fabrics, particularly in high-temperature applications.

Unfortunately, the material can only be extruded with difficulty in monofilament form in the size range commonly used in dryer fabrics. Also during weaving the pure material is subject to frequent warp breakages due to its lack of toughness and is prone to scraping in the loom heddles and reed dents, all of which renders pure polyphenylene sulphide difficult for heavy industrial weaving.

The addition of a heat-stabilized polyamide 66 to the polyphenylene sulphide before extrusion has greatly alleviated these problems. Experiments in a range of blends has confirmed the following important results:
1. the addition of polyamide 66 acts as a processing aid, which makes the commercial extrusion of the blend a more viable process;
2. "toughness" is significantly enhanced. For example, the addition of 6% by weight of heat-stabilized polyamide 66 increased the measured knot toughness by a factor of seven times. This property is determined by subjecting a strand, which contains a simple overhand knot, to tensile pull and producing a resulting load-elongation diagram. The area under the curve is a measure of knot toughness;
3. full hydrolytic degradation resistance is retained;
4. there is no sacrifice in tensile strength when the polyamide is added to the pure polyphenylene sulphide;
5. subsequent pilot plant and commercial weaving in a wide range of dryer fabric designs, including those requiring high weaving tensions and high pick counts, confirms that the use of the polyphenylene sulphide/6% polyamide blend in warp strands of dryer fabrics reduced warp breakage and scraping to an acceptable level;
6. increasing the polyamide 66 from 6% to 20% increases the toughness of the monofilament, however, the abrasion resistance decreases.

The means by which the additive improves toughness while preserving hydrolysis resistance is not entirely known, but the successful monofilaments are characterized by having the additive material present in small, discrete, elongated globules with the long axis parallel to the axis of the monofilament. These discrete globules are not connected to each other or to the outer boundaries of the monofilament, and are thus protected from the harsh environment of the end use application of the filament. In order to preserve the additive as discrete globules we have found that the melt viscosity of the added material must be higher than the melt viscosity of polyphenylene sulphide at the extrusion temperature and the amount of additive must be limited. Another factor to consider in choosing the additive is that it must not degrade during extrusion when it is temporarily exposed to the temperature required to melt the polyphenylene sulphide, the range being 285°C to 315°C. Some additives which satisfy the above mentioned requirements do not form globules because they are chemically incompatible with polyphenylene sulphide and react in unsuitable ways.

In our experiments in blending to date, we have found that heat-stabilized polyamide 66 is the only additive to polyphenylene sulphide which successfully imparts the quality of toughness to the resultant monofilament while preserving hydrolysis resistance. Other materials may be found which can also impart the same quality to the blend. Some factors which are important in choosing additives are: a higher viscosity at extrusion temperature than polyphenylene sulphide, chemical compatability, resistance to heat degradation during extrusion.

All types of dryer fabrics having monofilaments in the machine direction will benefit in resistance to hydrolysis from this invention. Three preferred constructions utilizing rectangular machine direction components are described below but the invention is not limited to these constructions.
Figs. 2 and 2A depict a plain weave dryer fabric 30 representative of a single-layer dryer fabric used in the papermaking industry. In Figs. 2 and 2A numeral 31 denotes consecutive warp strands made from polyphenylene sulphide or a blend of polyphenylene sulphide and polyamide 66 flattened to an essentially rectangular cross-section and numeral 32 represents consecutive weft strands. In this structure each warp strand 31 passes over a first weft strand 32, under the second weft strand, over the third and so on. Similarly, the adjacent warp strand passes under the first weft, over the second, under the third and so on.
Figs. 3 and 3A depict a four-shaft eight-repeat duplex-weave dryer fabric 40, which is a type commonly used in the papermaking industry. In Figs. 3 and 3A numerals 41, 42, 43 and 44 are consecutive warp strands, made from polyphenylene sulphide or a blend of polyphenylene sulphide and polyamide 66, flattened to an essentially rectangular cross-section. The weft is paired in two layers and numbered 48 to 57 as shown. In this woven structure a warp strand 41 passes in sequence over a pair of weft strands 50-51, between the next pair 52-53, under the third pair 54-55, between the fourth pair 56-57, and so on. The next consecutive warp strand 42 passes between the first pair of weft strands 50-51, over the second pair, between the third pair and under the fourth pair. Similarly, the third and fourth consecutive warp strands 43 and 44 are woven commencing under and between the first pair of weft strands respectively.
Fig. 4 depicts the essentially rectangular cross-section of the polyphenylene sulphide or polyphenylene sulphide/polyamide blend warp strands. Such strands may be produced by rolling round monofilament strands, or by slitting film, or, in the preferred embodiment by melt-extruding through a specially shaped die. The flatness ratio a:b of the preferred embodiment shown in Fig. 4 is 2:1 and is preferably between 1.5:1 and 2.5:1 for the woven dryer fabric embodiments.
Figs. 5 and 5A depict a spiral construction dryer felt 60 comprising a plurality of helical S-coils 61 joined together with adjacent Z-coils 62 by means of hinge pins 63. The designations 'S' and 'Z' indicate the direction of twist, following the convention in the textile industry. The coils 61, 62 are wound using polyphenylene sulphide or polyphenylene sulphide/polyamide blend strand material of essentially rectangular cross-section with a flatness ratio a:b of 2:1 as shown in this preferred embodiment. In this construction a range of flatness ratios between 1.1:1 and 2.5:1 can be used.

The woven dryer fabric of the present invention has a warp count preferably in the range of 25 to 80 strands per inch (2.5 cm). Warp strands are made by polyphenylene sulphide or a blend of polyphenylene sulphide and polyamide 66. The flattened warp strands of the invention will have major axis measurements in the range of 0.0125" to 0.050" (0.32 to 1.27 mm). With respect to weft it is not intended to limit the material utilized to monofilaments. Since in the fabric of the invention the weft strands are non-loadbearing, other materials resistant to high temperature and hydrolytic degradation may be utilized, for example composite strands incorporating asbestos or fibreglass.

The dryer fabric of spiral construction, which is another embodiment of the invention, utilizes helical coils made from polyphenylene sulphide or a blend of polyphenylene sulphide and heat-stabilized polyamide 66 up to 20% by weight of polyamide 66. Hinge pins may be made from the same material or alternatively from other temperature resistant materials such as the composite constructions already mentioned.

In the preferred embodiments above, rectangular shaped monofilaments have been used, but round monofilaments and other cross-sectional shapes may also be used provided they are made from the material of this invention. We have found that woven fabrics made with rectangular warp strands of pure polyphenylene sulphide, and in a different test with warp strands made from a 6% blend of polyamide 66 and polyphenylene sulphide have superior resistance to distortion compared to equivalent fabrics made with monofilament polyester warp material. Thus, the invention can be used to improve the distortion resistance of fabrics made with round monofilaments which is normally troublesome.

## Claims

1. A dryer fabric for use in a dryer section of a paper machine wherein at least the machine direction components of the fabric are monofilaments made from polyphenylene sulphide or a blend of polyphenylene sulphide with heat-stabilized polyamide 66, said polyamide 66 being present in the range of up to about 20% by weight.

2. A dryer fabric as claimed in claim 1 wherein said polyphenylene sulphide is blended with about 6% by weight of heat stabilized polyamide 66.

3. A dryer fabric as claimed in claim 1 wherein said machine direction components are warp strands in a woven dryer fabric.

4. A dryer fabric as claimed in claim 3 wherein said warp strands are flattened warp strands having an essentially rectangular cross-section with the long axis of the rectangle lying in the plane of said fabric.

5. A dryer fabric as claimed in claim 4 wherein said woven dryer fabric has flattened warp strands having an essentially rectangular cross-section with a flatness ratio between 1.5:1 and 2.5:1.

6. A dryer fabric as claimed in claim 1 wherein said said machine direction components comprise a plurality of helical coils connected together by hinge pins.

7. A dryer fabric as claimed in claim 6 wherein the monofilament of said helical coils has an essentially rectangular cross-section when viewed in the machine direction with the long axis of the rectangle lying in the plane of said fabric.

8. A dryer fabric as claimed in claim 7 wherein said rectangular cross-section has a flatness ratio between 1.1:1 and 2.5:1.

9. A dryer fabric as claimed in claim 1 wherein said monofilaments are made from polyphenylene sulphide and an additive which imparts toughness to the monofilament while preserving the hydrolysis resistance inherent in polyphenylene sulphide, said additive having characteristics of a higher melt viscosity than the polyphenylene sulphide at extrusion temperatures, resistance to thermal degradation at extrusion temperatures, and chemical compatibility with the polyphenylene sulphide, and wherein said additive is present in small discrete elongated globules with the long axis of said globules parallel to the axis of the monofilament.

10. A dryer fabric as claimed in claim 9 wherein said globules are not connected to the outer boundaries of the monofilament.

11. A dryer fabric as claimed in claim 3 wherein said fabric has a warp count in the range of 25 to 80 strands per 2.54 cm (per inch).

12. A monofilament made from a blend of polyphenylene sulphide and an additive, said additive imparting improved toughness to the resulting monofilament without substantially reducing its hydrolysis resistance, said additive being added to the polyphenylene sulphide in the range of 1% to 20% by weight and having the characteristics of
- higher viscosity at extrusion temperatures than polyphenylene sulphide;
- resistance to degradation during extrusion;
- chemical compatability with polyphenylene sulphide;
- being present in the monofilament in small discrete elongated globules with the long axis of said globules parallel to the axis of the monofilament.

13. A monofilament as in claim 12 wherein the additive is heat-stabilized polyamide 66.

14. A monofilament as in claim 13 wherein the heat-stabilizing polyamide 66 comprises about 6% by weight of the polyphenylene sulphide.

15. A monofilament as in claim 12 having a flattened essentially rectangular cross-section with an axis ratio between 1.1 to 1 and 3 to 1.

16. A monofilament as in claim 15 with an axis ratio of about 2 to 1.

17. A monofilament as claimed in claim 15 having a major axis measurement in the range from 0.32 to 1.27 mm (0.0125 to 0.050 inches).

18. A monofilament as in any one of the preceding claims 12 to 17 wherein said discrete globules are not connected to the outer boundaries of the monofilament.

19. A synthetic industrial fabric comprising a fabric woven from monofilaments or a fabric composed of a plurality of helically coiled monofilaments connected together by hinge pins, wherein said monofilaments comprise monofilaments in accordance with one of claims 12 or 13.

## Patentansprüche

1. Trockengewebe zur Verwendung in einer Trockenpartie einer Papiermachine, bei der mindestens die in Bearbeitungsrichtung verlaufenden Bestandteile des Gewebes Einzelfäden aus Polyphenylensulphid oder einem Gemisch aus Polyphenylensulphid mit wärmestabilisiertem Polyamid 66 sind, wobei das Polyamid 66 im Bereich bis zu 20 Gew.-% vorhanden ist.

2. Trockengewebe nach Anspruch 1, bei dem das Polyphenylensulphid mit etwa 6 Gew.-% wärmestabsilisiertem Polyamid 66 gemischt ist.

3. Trockengewebe nach Anspruch 1, bei dem die in Bearbeitungsrichtung verlaufenden Komponenten Kettfäden in einem gewebten Trockengewebe sind.

4. Trockengewebe nach Anspruch 3, bei dem die Kettfäden abgeflachte Kettfäden mit einem im wesentlichen rechtwinkligen Querschnitt sind, wobei die längere Achse des Rechtecks in der Ebene des Gewebes liegt.

5. Trockengewebe nach Anspruch 4, bei dem das gewebte Trockengewebe abgeflachte Kettfäden mit einem wesentlichen rechtwinkligen Querschnitt mit einem Abflachungsverhältnis zwischen 1,5:1 und 2,5:1 besitzt.

6. Trockengewebe nach Anspruch 1, bei dem die in Bearbeitungsrichtung verlaufenden Komponenten eine Vielzahl von miteinander durch Gelenkstifte verbundene Wendelwicklungen umfaßt.

7. Trockengewebe >nach Anspruch 6, bei dem der Einzelfaden der Wendelwicklungen in Bearbeitungsrichtung gesehen einen im wesentlichen rechtwinkligen Querschnitt bestizt, wobei die lange Achse des Rechtecks in der Gewebeebene liegt.

8. Trockengewebe nach Anspruch 7, bei dem das Abflachungsverhältnis des rechtwinkligen Querschnitts zwischen 1,1:1 und 2,5:1 liegt.

9. Trockengewebe nach Anspruch 1, bei dem Einzelfäden aus Polyphenylensulphid und einem Zusatz hergestellt sind, der dem Einzelfaden Zähigkeit verleiht unter Aufrechterhaltung des dem Polyphenylensulphid eigenen Hydrolyse-Festigkeit, wobei das Additiv Eigenschaften einer höhren Schmelzviskosität als das Polyphenylensulphid bei Extrusionstemperaturen, Widerstand gegen thermischen Abbau bei Extrusionstemperaturen und chemische Verträglichkeit mit dem Polyphenylensulphid aufweist, und wobei der Zusatz als kleine diskrete längliche Kügelchen vorhanden ist, mit der Längsachse der Kügelchen parallel zur Achse des Einzelfadens.

10. Trockengewebe nach Anspruch 9, bei dem Kügelchen nicht mit der Außenbegrenzung des Einzelfadens in Verbindung sind.

11. Trockengewebe nach Anspruch 3, bei dem das Gewebe eine Kettzahl im Bereich von 25 bis 80 Kettfäden pro 2,54 cm (pro inch) besitzt.

12. Einzelfaden aus einem Gemisch aus Polyphenylensulphid und einem Zusatz, der dem sich ergebenden Einzelfaden verbesserte Zähigkeit verleiht, ohne seine Hydrolyse-Festigkeit wesentlich zu verringern, wobei der Zusatz zu dem Polyphenylensulphid im Bereich von 1 bis 20 Gew.-% hinzugefügt ist und die Eigenschaften besitzt.
- höhere Viskosität bei Extrusionstemperaturen als Polyphenylensulphid;
- Widerstand gegen Abbau während der Extrusion;
- chemische Verträglichkeit mit Polyphenylensulphid, und
- in dem Einzelfaden in kleinen diskreten länglichen Kügelchen vorhanden ist, wobei die Längsachse der Kügelchen parallel zur Achse des Einzelfadens liegt.

13. Einzelfaden nach Anspruch 12, bei dem der Zusatz wärmestabilisiertes Polyamid 66 ist.

14. Einzelfaden nach Anspruch 13, wobei das wärmestabilisierte Polyamid 66 etwa 6 Gew.-% des Polyphenylensulphid umfaßt.

15. Einzelfaden nach Anspruch 12 mit einem abgeflachten im wesentlichen rechtwinkligen Querschnitt mit einem Achsenverhältnis zwischen 1,1 zu 1 und 3 zu 1.

16. Einzelfaden nach Anspruch 15 mit einem Achsenverhältnis von etwa 2 zu 1.

17. Einzelfaden nach Anspruch 15 mit einer Abmessung der großen Achse im Bereich von 0,32 bis 1,27 mm (0,0125 bis 0,050 inch).

18. Einzelfaden nach einem der vorangehenden Ansprüche 12 bis 17, bei dem die diskreten Kügelchen nicht mit der Außenbegrenung des Einzelfadens in Verbindung sind.

19. Synthetisches Industriegewebe mit einem aus Einzelfäden gewebten Gewebe oder einem Gewebe, das aus einer Vielzahl von wendelförmig gewickelten Einzelfäden zusammengesetzt ist, die durch Gelenkstifte miteinander verbunden sind, wobei die Einzelfäden Einzelfäden nach einem der Ansprüche 12 oder 13 umfassen.

## Revendications

1. Toile de séchage pour l'utilisation dans une section de séchage d'une machine à papier, dans laquelle au moins les composants de la toile suivant la direction de la machine sont des monofilaments faits de poly(sulfure de phénylène) ou d'un mélange de poly(sulfure de phénylène) avec un polyamide 66 stabilisé en température, ledit polyamide 66 étant présent dans la plage de jusqu'à 20% en poids environ.

2. Toile de séchage selon la revendication 1, dans laquelle ledit poly(sulfure de phénylène) est mélangé avec environ 6% en poids de polyamide 66 stabilisé en température.

3. Toile de séchage selon la revendication 1, dans laquelle lesdits composants suivant la direction de la machine sont des brins de chaîne d'une toile de séchage tissée.

4. Toile de séchage selon la revendication 3, dans laquelle lesdits brins de chaîne sont des brins de chaîne aplatis ayant une section transversale substantiellement rectangulaire avec le grand axe du rectangle étendu dans le plan de ladite toile.

5. Toile de séchage selon la revendication 4, dans laquelle ladite toile de séchage tissée possède des brins de chaîne aplatis ayant une section transversale substantiallement rectangulaire avec un rapport d'aplatissement entre 1,5:1 et 2,5:1.

6. Toile de séchage selon la revendication 1, dans laquelle lesdits composants suivant la direction de la machine comportent une pluralité d'enroulements hélicoïdaux liés ensemble par des broches.

7. Toile de séchage selon la revendication 6, dans laquelle le monofilament desdits enroulements hélicoïdaux possède une section transversale substantiellement rectangulaire vu suivant la direction de la machine avec le grand axe du rectangle étendu dans le plan de ladite toile.

8. Toile de séchage selon la revendication 7, dans laquelle ladite section transversale a un rapport d'aplatissement entre 1,1:1 et 2,5:1.

9. Toile de séchage selon la revendication 1, dans laquelle lesdits monofilaments sont faits de poly(sulfure de phénylène) et d'un additif qui confère de la dureté au monofilament tout en conservant la résistance à l'hydrolyse propre au poly(sulfure de phénylène), ledit additif possédant des caractéristiques de viscosité de fusion supérieure à celle du poly(sulfure de phénylène) aux températures d'extrusion, de résistance à la dégradation thermique aux températures d'extrusion, et de compatibilité chimique avec le poly(sulfure de phénylène), et dans laquelle IequeI additif est présent en globules discrets allongés avec le grand axe desdits globules parallèles à l'axe du monofilament.

10. Toile de séchage selon la revendication 9, dans laquelle lesdits globules ne sont pas liés aux frontières extérieures du monofilament.

11. Toile de séchage selon la revendication 3, dans laquelle ladite toile possède un compte en chaîne dans la gamme de 25 à 80 brins par 2,54 cm (par inch).

12. Un monofilament fait d'un mélange de poly(sulfure de phénylène) et d'un additif, ledit additif conférant une dureté augmentée au monofilament résultant sans réduire sensiblement sa résistance à l'hydrolyse, ledit additif étant ajouté au poly(sulfure de phénylène) dans la plage de 1 % à 20% en poids et possédant les caractéristiques de
- viscosité supérieure à celle du poly(sulfure de phénylène) aux températures d'extrusion;
- résistance à la dégradation pendant l'extrusion;
- compatibilité chimique avec le poly(sulfure de phénylène);
- être présent dans le monofilament en petits globules allongés discrets, avec le grand axe desdits globules parallèles à l'axe du monofilament.

13. Monofilament selon la revendication 12, dans lequel l'additif est un polyamide 66 stabilisé en température.

14. Monofilament selon la revendication 13, dans lequel le polyamide 66 stabilisé en température représente environ 6% en poids du poly(sulfure de phénylène).

15. Monofilament selon la revendication 12, ayant une section transversale substantiellement rectangulaire avec un rapport d'axe entre 1,1 à 1 et 3 à 1.

16. Monofilament selon la revendication 15, avec un rapport d'axe d'environ 2 à 1.

17. Monofilament selon la revendication 15, ayant une dimension de grand axe dans la plage 0,32 à 1,27 mm (0,0125 à 0,050 inches).

18. Monofilament selon une quelconque des revendications précédentes 12 à 17, dans ledit lesdits globules discrets ne sont pas liés aux frontières extérieures du monofilament.

19. Toile industrielle synthétique comprenant une toile tissée à partir de monofilaments, ou une toile composée d'un pluralité de monofilaments enroulés en hélice et liés ensemble par des broches, dans laquelle lesdits monofilaments comprennent des monofilaments selon l'une des revendications 12 et 13.
